

Nov. 13, 1928.

1,691,029

A. F. BANDUR

CONDUCTOR FOR THE TRANSMISSION OF ELECTRICAL ENERGY  
AND METHOD OF PRODUCING THE SAME

Filed April 22, 1924

*Fig. 1*



*Fig. 2*



*Inventor  
Adolph F. Bandur  
by H. A. Patterson  
Atty.*

## UNITED STATES PATENT OFFICE.

ADOLPH FRANCIS BANDUR, OF BEEWYN, ILLINOIS, ASSIGNOR TO WESTERN ELECTRIC COMPANY, INCORPORATED, OF NEW YORK, N. Y., A CORPORATION OF NEW YORK.

CONDUCTOR FOR THE TRANSMISSION OF ELECTRICAL ENERGY AND METHOD OF PRODUCING THE SAME.

Application filed April 22, 1924. Serial No. 708,128.

This invention relates to conductors for the transmission of electrical energy and methods of producing the same, and more particularly to composite signalling conductors having an external layer of material of high permeability for the purpose of increasing the inductance of the conductor, the electrical characteristics of the material being determined to some extent by heat treatment.

One manner of increasing the inductance of a conductor employed for the transmission of alternating current is to wrap the conductor spirally with a layer of wire or tape of magnetic material. This method is known in the art as continuous inductive loading as distinguished from lump loading by means of coils distributed along the conductor. Until recently iron has been considered to be the only material available for continuous loading. It has been discovered, however, that a more suitable material may be produced in the form of an alloy of nickel and iron. When these two metals are in proper proportions and the alloy is given proper heat treatment, a material having very high permeability at low magnetizing forces is obtained. For a full disclosure of the metallurgical and electrical characteristics of this alloy and its heat treatment, reference is made to the patents of Gustave W. Elmen, 1,586,884, issued June 1, 1926; Oliver E. Buckley, 1,586,874, issued June 1, 1926, and Gustave W. Elmen, 1,586,887, issued June 1, 1926.

One method of applying the alloy loading material above described to a composite signalling conductor is that described in Patent 1,537,575, issued May 12, 1925, in which the loading material is applied in the form of tape wrapped around the conductor and subjected to the requisite heat treatment while wrapped thereon.

It has been found that when this alloy loading material is subjected to stresses or strains that the permeability thereof is materially lowered and that in some cases these deleterious stresses or strains occur during the heat treatment of the loading material and are due to the construction of the composite conductor.

An object of this invention is to provide a composite electrical conductor so treated that when it has been wrapped with a mag-

netic material which requires heat treatment, the magnetic material will not be subjected to any deleterious stresses or strains during such heat treatment thereof.

Another object of the invention is to provide a method of treatment for the composite conductor prior to the application of the magnetic material thereto.

In accordance with the invention the composite conductor is coated with a non-combustible lubricating material which will permit relative movement between the composite conductor and the magnetic loading tape during the heat treatment of the latter without subjecting the loading tape to deleterious stresses or strains.

Other objects and advantages of the invention will appear from the following detailed description and will be particularly pointed out in the appended claims.

In the accompanying drawings,

Fig. 1 is a fragmentary side elevation of a composite conductor made in accordance with the invention, part of the alloy loading tape being cut away to more clearly show the composite conductor and the lubricating material applied thereto, and

Fig. 2 is a vertical sectional view of Fig. 1.

In carrying out the invention a composite conductor is produced consisting of a central conductor 5, around which a plurality of copper segmental strips 6, preferably six in number, are stranded so that they lie flat thereagainst. The composite conductor thus produced is then coated with a thin coating of non-combustible lubricating material 7, preferably powdered mica, as shown in the drawing, the said coating having a thickness of approximately .005".

The non-combustible coating may be applied by drawing the composite conductor through a receptacle containing the powdered mica or applied in any other suitable manner.

The alloy loading material 8 is then wrapped around the coated composite conductor by any suitable means, but preferably by the method and apparatus disclosed in Patent 1,565,652, issued December 15, 1925.

The central copper conductor 5 and the segmental strips 6 have a higher coefficient of elongation than the alloy tape 8. Measuring a plurality of samples of the composite

conductor and the alloy tape, the former has been found to have a coefficient of elongation from 11 to 53 per cent. higher than that of the alloy tape. Due to this difference, 5 unless precautions are taken to prevent it, the natural tendency of the composite conductor to expand more rapidly than the alloy tape will cause the latter to be subjected to deleterious stresses and strains during the 10 heat treatment thereof. The difficulty of obviating these stresses and strains is increased, since during the heat treatment of the loaded conductor it is raised from room temperature to 1530° F. during approximately 47 seconds 15 time.

Due to the fact that the strips 6 are relatively flat, upon being stranded around the central conductor 5, they do not present a true cylindrical surface because the edges 20 of the strips do not lie flat against the central conductor, but present spiral ridges. During the heat treatment the alloy tape 8 and copper strips 6 tend to move relatively to each other due to their different coefficients 25 of elongation, and unless some means is provided to prevent it, the ridges formed by the strips 6 cause a sticking between the said strips and the alloy tape 8, subjecting the latter to deleterious stresses and strains, 30 both during the heating and cooling thereof. However, when powdered mica is coated over the ridges formed by the strips 6, a non-combustible lubricant is provided which prevents sticking between the strips 6 and alloy 35 tape 8 and permits relative movement between them during the heating and cooling thereof, incident to the heat treatment of the alloy tape. Where the strips 6 and alloy tape 8 are free to move relatively to each other 40 during the heat treatment, the alloy tape 8 is not subjected to deleterious stresses or strains at a time when such stresses or strains have a very great effect upon its electrical characteristics.

45 What is claimed is:

1. A loaded signalling conductor comprising a central conductor, a coating of material thereon which will act as a separator and which will not be consumed on being subjected to heat treatment, and a magnetic loading material wrapped around said central conductor, said loading material requiring heat treatment to give it a desired electrical characteristic.
5. 2. A loaded signalling conductor comprising a central conductor, a coating of powdered mica, and a magnetic loading material wrapped around said central conductor, said loading material requiring heat treatment to give it a desired electrical characteristic.
- 10 3. A loaded signalling conductor comprising a composite metallic strand consisting of a metallic wire wrapped with metallic strip, a coating of material on said composite strand

which will act as a separator and which will 65 not be consumed on being subjected to heat treatment, and a magnetic loading material wrapped around said composite strand, said loading material requiring heat treatment to give it a desired electrical characteristic.

70 4. A loaded signalling conductor comprising a composite strand consisting of a metallic wire wrapped with relatively flat metallic strip, a coating of mica on said metallic strip, and a magnetic loading material wrapped 75 around said composite strand, said loading material requiring heat treatment to give it a desired electrical characteristic.

80 5. The method of loading a signalling conductor with magnetic material requiring heat treatment to give it a desired electrical characteristic, consisting in coating the central conductor with a separating material, wrapping the loading material around the said coated conductor, subjecting the thus assembled conductor to heat treatment, and preventing the destruction of the separating material by the heat treatment.

85 6. The method of loading a signalling conductor with magnetic material requiring heat treatment to give it a desired electrical characteristic, consisting in wrapping a metallic wire with relatively flat metallic strip, coating the said strip with a separating material, wrapping the loading material around the coated composite strand, annealing the conductor, and maintaining the separating material intact during the annealing process.

90 7. The method of loading a signalling conductor with magnetic material which requires heat treatment to give it a desired electrical characteristic, which consists in stranding a plurality of relatively flat copper strips around a copper wire, coating the outer surface of the strips with powdered mica, and then wrapping the magnetic loading material in the form of relatively flat metallic tape around the coated composite strand, annealing the conductor, and retaining the mica in its original form.

95 8. The method of preventing a decrease in the permeability of a magnetic material applied to an electrical conductor, which consists in applying a layer of separating material to said conductor prior to wrapping the magnetic material thereon, annealing said magnetic material, and retaining the separator between the conductor and the magnetic material by means of a separating material due to its not being consumed.

100 9. A loaded signaling conductor comprising a central conductor, a magnetic loading material wrapped around said central conductor, said loading material requiring heat treatment to give it a desired electrical characteristic, and a separator located between said central conductor and said magnetic loading material, which will not be consumed

upon being subjected to the high temperature incident the heat treating of the magnetic loading material.

10. The method of preventing a decrease in permeability of a magnetic material applied to an electrical conductor, which consists in applying a non-combustible separator

to the conductor prior to application of the magnetic material thereto, annealing said magnetic material, and retaining the separator intact during the annealing process. 10

In witness whereof, I hereunto subscribe my name this 11th day of April, A. D. 1924.

ADOLPH FRANCIS BANDUR.